

## UNITED STATES PATENT OFFICE

2,658,840

PROCESS FOR THE MANUFACTURE OF  
LAMINATESJoseph C. Perry, Los Angeles, Calif., assignor to  
Agrashell, Inc., Los Angeles, Calif., a corpora-  
tion of DelawareNo Drawing. Application July 18, 1950,  
Serial No. 174,580

9 Claims. (Cl. 117—111)

1

This invention relates to the manufacture of laminates including plywood and more specifically to a gluing procedure in the production of laminates involving a process capable of utilizing more highly filled phenol-formaldehyde glue mixes.

Under present commercial practice, plywood of two principal types are produced, namely all-weather plywood and interior plywood from either hardwood or softwood. The former employs substantially exclusively a phenol-formaldehyde resin glue emulsion which is relatively expensive as compared to the cost of other plywood glues. Interior plywoods are prepared almost exclusively from proteinous glues and the boards produced therefrom do not possess the greater strength and high weather and mold resistant properties of the exterior plywood. The glue mixes used for both types of plywood are composed of glue, a ligno-cellulose or other extender and water.

It has been realized for some time that it is highly desirable to find some means whereby plywood for interior use can be produced utilizing phenol-formaldehyde resin glues at a price comparable to that at which the interior plywood is prepared. Several operators heretofore attempted to accomplish this desirable end by the addition of a larger quantity of a suitable filler, and a great deal of experimental work has been conducted using different fillers and variously modified resins or additions, all without success.

Modern plywood plants are highly mechanized and operate on the straight line production basis in which each unit operation dovetails into the next and a continuous flow of finished product is discharged from the end of assembly lines. The glue spreading machine which applies the glue mix to the surface of the prepared boards prior to the time the plies are assembled for loading into steam heated platen presses for final curing, is one of these units which must be operated on a carefully controlled time schedule.

The glue mix must possess a number of properties under constant control. It must remain tacky for the period required for assembling the plies and it must cure and set rapidly to provide for hardening within the required curing time cycle. The glue mix also must remain at a constant consistency sufficient to avoid any appreciable variation in the thickness of the glue film applied as the consumption of the batch of glue proceeds. Therefore, very little variation in the resin-extender-water ratio has been permissible.

The conventional glue mix for producing ex- 55 manner or means by which the glue mix is

2

terior plywood is composed of phenol-formaldehyde resin glue emulsion (42% solid) with vegetable shell flour extender and water in the weight ratio of 5:1:1. If the quantity of the extender is appreciably increased, the consistency of the glue mix changes and becomes more viscous and the quantity of glue applied by the spreader increases and thus it is not only wasted but reduces the bond strength of the plywood. If only an amount of water is added to this highly extended mix sufficient to obtain the required consistency or viscosity for initial application, the glue mix changes in consistency on the spreader before the glue can be applied. If still greater quantities of water are employed to prevent this excess thickening, the resulting glue would be thrown off the spreader rolls due to low initial viscosity, would cause the extender to separate from the resin binder and would cause the boards to "blow" in the press due to excessive steam release.

Accordingly, an object of the present invention is to provide a process for the production of a plywood using phenol-formaldehyde resin glue, of a quality superior to that of conventional interior plywood at a cost competitive with or cheaper than the cost of producing such interior plywood bonded with proteinous glues.

In its primary embodiment, the invention involves (1) preparing a glue mix containing phenol-formaldehyde resin glue and an extender in larger proportions than has heretofore been possible or with an amount of extender reducing the over-all cost of the glue mix to a figure competitive with that of conventional glue mixes for interior plywood production, and (2) cooling the resulting glue mix and maintaining the same at a temperature of from about 35° to 75° F. until it is applied to the hard or soft wood veneers (laminae). Through this simple procedure of temperature control, the consistency and viscosity requirements are retained and the straight line production can be continued as if conventional glue mixes were being employed under most favorable conditions. The permissible range of operable temperatures varies somewhat with the nature of the extender and the ratio of the same to the resin solids of the glue employed. Higher extender ratios ordinarily require lower temperatures. A temperature within the range of about 45° to 55° gives best results in ordinary operations and even when very highly filled resin mixes are being applied.

The instant invention is independent of the manner or means by which the glue mix is

cooled to the desired temperature. It may be cooled in the conventional mixing tank, in the glue well or on the glue spreader rolls. The cooling may be accomplished through the insertion of cooling coils in the tank or well or by cooling jackets surrounding the tank or well. Instead of cooling the glue mix within said containers it may be circulated through coils immersed in a cooling medium after which it is returned to the containers. Regardless of the apparatus employed, the cooling means may be and is preferably thermostatically controlled such that the conditions are held constant throughout continuous operation.

If the cooling of the glue mix is carried out in the mixing tank, then the temperature to which it is cooled should be somewhat lower to allow for the increase in temperature which will occur during the transfer of the glue mix from the tank, through the well, over the rolls and to the boards being treated.

Experimentation has indicated that glue mixes are operable which contain proportions by weight between about 15 to 25% resin solids and from 15 to about 40% or more ligno-cellulose filler. In such mixes the remainder is water and will ordinarily be present in the amount of from 35 to 70%.

In accordance with prior straight line production practice, it has not been practically possible or safe to employ glue mixes containing more than five-tenths of one part filler by weight for each part phenol-formaldehyde resin solids. Through the temperature control process of the present invention, satisfactory operations have been conducted employing from six-tenths to two or more parts of the filler per part resin solids.

The process of the invention is applicable to the conventional phenol-formaldehyde resin glue emulsions supplied by various manufacturers. The use with the glue of various recommended accelerators, hardeners, alkalizing agents or other aids does not prevent the advantages of the instant temperature control process from being realized.

To illustrate examples of glue mixes found suitable for use in the practice of the present process, a number of compositions are set out in the table below, the ratios given being in parts by weight. The resin employed was an aqueous emulsion of phenol-formaldehyde resin having 42% solids as "Plyophen." The flour used was walnut shell flour, as "Glufil."

|          | Glue Mix Ratio |       |       | Caus-<br>tic <sup>1</sup> | Per-<br>cent<br>Resin<br>Solids | Per-<br>cent<br>Water | Per-<br>cent<br>Flour |
|----------|----------------|-------|-------|---------------------------|---------------------------------|-----------------------|-----------------------|
|          | Resin          | Flour | Water |                           |                                 |                       |                       |
| (a)..... | 5              | 1½    | 2     | ½                         | 23                              | 54                    | 16.6                  |
| (b)..... | 5              | 2     | 2½    | -----                     | 22.1                            | 56.8                  | 21.0                  |
| (c)..... | 5              | 1½    | 3     | -----                     | 22.1                            | 62.1                  | 15.8                  |
| (d)..... | 5              | 1½    | 3     | ½                         | 21.0                            | 59.0                  | 15.0                  |
| (e)..... | 5              | 2     | 3     | -----                     | 21.0                            | 59.0                  | 20.0                  |
| (f)..... | 5              | 2     | 3     | ½                         | 20.0                            | 56.3                  | 19.0                  |
| (g)..... | 5              | 3     | 4½    | -----                     | 17.1                            | 58.3                  | 24.5                  |

<sup>1</sup> Sodium hydroxide or carbonate.

The cost of the more highly filled glue mixes illustrated in these examples is appreciably less than the cost of conventional proteinous glue used in the preparation of interior plywood. The presence of the larger proportions of the low cost extender more than over balances the higher glue cost of the phenol-formaldehyde resin.

The addition of viscosity controlling agents as bentonite, lecithin, carboxy methyl cellulose

or soaps may be resorted to in order to obtain any required initial viscosity. Furthermore, the preparation of the mixes may be facilitated by passage through a roller mill or a homogenizer or other device to assist the wetting of the filler and to obtain and maintain better dispersion of the filler throughout the mix.

Although the present invention is directed primarily to the production of highly filled phenol-formaldehyde resin glue mixes, the cooling step of the present invention may be advantageously employed in the application of other resin glues similarly affected by heat when highly filled. Also the process may be used in the manufacture of conventional exterior plywood wherein the resin emulsion-extender-water ratio is ordinarily 5:1:1. The proper application or utilization of this glue mix sometimes gives considerable trouble during changes in humidity and temperature occurring from day to day. The control of the temperature of this glue mix in accordance with the present procedure eliminates this difficulty.

Manufacturers of exterior plywood generally know that the ratio of binder solids in the glue mixes they employ is higher than is essential to obtain adequate bond strength, but they have not been willing to use a lesser proportion of glue in view of the difficulties and delays 25 encountered when the periodic changes in atmospheric moisture and temperature conditions occur. With the utilization of the process of the present invention, a greater proportion of filler can be employed without sacrificing the high bonding qualities required of exterior plywood.

Whereas the filler preferably employed in the glue mixes of the invention is walnut shell flour, a great variety of other nut and vegetable shell flours can be used with good success. Other 30 ligno-cellulose fillers can be used for special purposes, as redwood bark flour, ligno-cellulose products derived from the manufacture of furfural, and fine particle size lignin resins themselves. The temperature control procedure is effective even when inorganic fillers are employed such as fine particle size clay.

#### EXAMPLE

A glue mix was prepared by stirring together 50 five parts phenol-formaldehyde resin emulsion, two parts walnut shell flour filler and two and one-half parts water. This glue mix was placed in the reservoir of a spreader and subjected to the action of the spreader rolls for one-half 55 hour during which the reservoir was cooled and the glue mix maintained at a temperature of 49° F. In a test, the viscosity of the resulting mass as 25° C. was 290 centipoises as compared with 230 centipoises measured at the same temperature, of the original mix immediately after its formation. This change of 60 centipoises is inconsequential and small in comparison with the change which occurs when no control over the temperature is exercised.

When another batch of this same glue mix 60 formulation was tested in the same manner except that the temperature was permitted to remain at 69° F. which approximates normal room temperature, its viscosity increased from 230 to 500 centipoises in the comparative tests conducted at 25° C. This increase in viscosity of 270 centipoises is high and of sufficient magnitude to prevent the glue from being employed in conventional straight line production operations.

The process of the present invention has a number of operational and economic advantages as follows:

A. Only an inconsequential change in viscosity occurs in the glue mix during the period of its application.

B. A more uniform distribution of glue mix over the veneers is obtained and the quantity of glue applied by the spreader rolls is more uniform for any given setting of the spreader rolls.

C. In those operations where adjustment of the doctor rolls of the spreader has heretofore been used as a means for compensating for viscosity changes in the glue mix, the necessity of such adjustment is eliminated.

D. A more uniform bond strength in the finished plywood is obtained for the primary reason that uneven glue spreads are eliminated.

E. The glue line costs are lowered due to more uniformly thin spreads.

F. Much larger quantities of filler can be employed which in turn effects a reduction in the glue line cost.

G. Greater quantities of water in the glue mix are permitted due to the fact that the low temperature increases the initial viscosity of the glue, and the addition of a small amount of water does not prevent the viscosity from coming within workable limits on the spreader rolls. In contrast thereto, if additional water were added to conventional glue mixes without temperature reduction the initial viscosity would be low and the glue would be thrown by centrifugal force from the high speed rolls of the spreader.

The process of the present invention is applicable to the straight line production of laminates other than plywood, as beams and a variety of specially shaped members.

It should be understood that the present invention is not limited to specific details herein given except where indicated to the contrary and that the invention extends to all equivalents which will occur to those skilled in the art upon consideration of the scope of the claims appended hereto.

I claim:

1. In the straight line production of plywood and other laminates from veneers, using a glue spreading machine having a glue reservoir, spreader and doctor rolls, the process which comprises mixing a thermosetting phenol-formaldehyde resin glue and water with a solid extender in weight proportions of 1 resin solids to .5 to about 2 of extender, cooling the resulting fusible glue mix while in said machine and maintaining its temperature at from 35° to 75° F. during the whole period the glue remains in said machine and until it is applied to the veneers whereby heat developed in the glue while in the machine is taken up and whereby satisfactory spreading qualities are retained and spreading the cooled glue on the veneers.

2. In the straight line production of plywood and other laminates from veneers, using a glue

spreading machine having a glue reservoir, spreader and doctor rolls, the process which comprises mixing a thermosetting phenol-formaldehyde resin glue and water with a solid extender in weight proportions of 1 resin solids to from .6 to about 2 of extender, withdrawing the heat developed in the glue due to the action of the rolls, by cooling the glue in the machine and maintaining its temperature at from 35° to 75° F. during the whole period the glue remains in the said machine and until it is applied to the veneers, whereby the viscosity of the glue in the machine is prevented from rising to a level which prevents successful application in the straight line operation, and spreading the cooled glue on the veneers.

3. In the straight line production of plywood and other laminates from veneers, using a glue spreading machine having a glue reservoir, spreader and doctor rolls, the process which comprises mixing a thermosetting phenol-formaldehyde

20 glue, water and a nut shell flour in weight proportions of 1 resin solids to .5 to about 2 of flour, cooling the resulting fusible glue mix while in said machine and maintaining its temperature

25 at from 35° to 75° F. during the whole period the glue remains in said machine and until it is applied to the veneers whereby heat developed in the glue while in the machine is taken up and whereby satisfactory spreading qualities are retained and spreading the cooled glue on the veneers.

4. The process defined in claim 1 wherein the extender is a lignocellulose material.

5. The process defined in claim 1 wherein the extender is a vegetable shell material.

6. The process defined in claim 1 wherein the extender is a nut shell extender.

7. The process defined in claim 1 wherein the extender is a nut shell extender, the proportion of resin solids to extender being in the range of 1 part of the former to .6 to about 2 parts of the latter, by weight.

8. The process defined in claim 1 with the further limitation that the temperature of the glue is maintained within the range of 45° to 55° F.

9. The process defined in claim 2 with the further limitation that the temperature of the glue is maintained within the range of 45° to 55° F.

JOSEPH C. PERRY.

#### References Cited in the file of this patent

#### UNITED STATES PATENTS

| Number       | Name       | Date          |
|--------------|------------|---------------|
| 55 1,716,665 | Redman     | June 11, 1929 |
| 2,414,415    | Rhodes     | Jan. 14, 1947 |
| 2,432,544    | Rhodes     | Dec. 16, 1947 |
| 2,473,145    | Hesselbart | June 14, 1949 |
| 2,489,336    | Spahr      | Nov. 29, 1949 |
| 60 2,574,784 | Heritage   | Nov. 13, 1951 |

#### OTHER REFERENCES

Forest Products Lab., Synthetic Resin Glues, Revised Mar. 1947, No. 1336.